

1

3,531,411  
LUBRICANT COMPOSITIONS

Albert Benson, Fairlawn, and Gerhart Karg, Pompton Lakes, N.J., assignors to Witco Chemical Company, Inc., New York, N.Y., a corporation of Delaware  
No Drawing. Filed Jan. 17, 1968, Ser. No. 698,397  
Int. Cl. C10m 3/02, 3/40  
U.S. Cl. 252—32.5

7 Claims

ABSTRACT OF THE DISCLOSURE

Chemically stable, aqueous-based lubricants, particularly for extreme pressure applications, having the combined properties of corrosion inhibition, low foam formation and anti-wear protection which compromise a solution containing minor amounts of an amine salt of phosphoric acid mono- and di-esters of condensation products or adducts of 1 mole of phenol with 1 to 6 moles of alkylene oxide.

This invention relates to novel lubricant compositions having improved properties in regard to chemical stability, corrosion inhibition, reduction of foaming tendencies, and anti-wear protection, for particular use in extreme pressure applications.

Lubricating compositions comprising oil base vehicles and lubricating compositions comprising water base vehicles and containing certain phosphate esters are known to the art and are disclosed in such U.S. patents as, for instance, Nos. 3,010,903; 3,169,923; 3,203,895; 3,297,098 and 3,310,489. In this last-mentioned patent, lubricating compositions are disclosed for use in metal working operations which may comprise water solutions containing from about 0.001 to about 20%, by weight, of various amine, notably triethanolamine, reaction products of certain phosphate esters, namely, phosphate mono- and di-esters of ethylene oxide adducts of hydroxyl compounds containing a hydrocarbon group having at least 9 aliphatic carbon atoms, said esters being exemplified by the phosphate mono- and di-esters of a 4 mol or 10 mol ethylene oxide adduct of nonylphenol, or phosphate mono- and di-esters of other nonionic surfactant ethylene oxide adducts of long chain alcohols or alkyl phenols containing, as indicated above a hydrocarbon group having at least 9 aliphatic carbon atoms. The patent emphasizes the importance of the presence of a hydrocarbon group having at least 9 aliphatic carbon atoms in the phosphate esters in order to obtain compositions which are useful for the purposes of the patent and wherein metal staining is avoided.

For certain metal working applications, such as using a lubricant as a synthetic cutting fluid, a certain combination of properties is of the utmost importance. These properties include stability at high temperature, high load-carrying capacity, protection against wear and corrosion and low foaming tendency. Low foam is a particularly important property for extreme pressure lubricants used in metalworking operations in order to insure the avoidance of blockage of the circulation system by air entrainment and to achieve good visibility at the work area.

In accordance with the present invention it has been discovered that aqueous solutions of amine salts of mono- or di-esters (and mixtures thereof) of phosphoric acid and a 1 to 6 mole ethylene oxide adduct of phenol have an unexpected combination of properties in regard to load carrying ability, low foaming, thermal stability and corrosion inhibition which render said solutions extremely effective as extreme pressure lubricants.

Generally, the phosphate esters utilized in the practice of the present invention can be prepared by reacting 1

2

mole of  $P_2O_5$  with 2 to 4.5 moles, preferably about 3 moles, of an adduct or condensation product of 1 to 6 moles, preferably about 3 moles, of ethylene oxide with 1 mole of phenol, using the type of procedure for the production of phosphate esters disclosed, for instance, in U.S. Pats. Nos. 2,441,295; 2,676,975; 2,701,258; 3,004,056 and 3,004,057; and German Pat. No. 696,317.

It has been found that, to achieve the desired characteristics, the phenol adduct from which the phosphate esters are prepared should contain no more than about 6 moles of ethylene oxide per mole of phenol. For example, the phosphate ester of an 8 mole ethylene oxide adduct of phenol has been found to exhibit relatively inferior properties in regard to foaming characteristics and load carrying ability when compared, for example, with the phosphoric acid ester of a 4 mole ethylene oxide adduct of phenol. Minor proportions of propylene oxide, for instance, can be used to replace a part of the ethylene oxide in making the adducts but, in general, the amount of propylene oxide utilized should not exceed about 20%, by weight, of the ethylene oxide. It is especially advantageous to use ethylene oxide solely as the alkylene oxide in making the adducts of phenol used in producing the phosphate esters which are employed in the compositions of the present invention.

The phosphate esters utilized in the practice of the present invention can be represented by the following formulae, (I) being the mono-ester and (II) being the di-ester:



where  $n$  is an integer from 1 to about 6, preferably 3 to 5 and particularly about 4. It will be noted that said esters are devoid of any hydrocarbon group containing at least 9 aliphatic carbon atoms.

The amine which is utilized as a reactant or to form a salt with the phosphate ester in the lubricating compositions of the present invention can be selected from a wide group so long as water-solubility of the product is obtained. Thus, said amines can be primary, secondary or tertiary, straight chain or branched chain, saturated or unsaturated, and can be of aliphatic, araliphatic or aromatic character. Of especial value are the hydroxyalkyl amines or alkanolamines, such as mono-, di- and tri-ethanolamine or mixtures thereof, particularly triethanolamine. Other illustrative examples of amines which can be used are dimethylamine; diethylamine; triethylamine; propylamine; monoisopropylamine, diisopropylamine, triisopropylamine, and commercial mixtures of said isopropylamines; butyl amine, amyl amine; monoisopropanolamine, diisopropanolamine, triisopropanolamine and commercial mixtures of said isopropanolamines; polyamines such as aminoethyl ethanolamine, ethylenediamine, diethylenetriamine, hydroxyethyl ethylenediamine, and hexamethylenediamine; hexylamine; cyclohexylamine; methylcyclohexylamine; alkyl alkanolamines such as ethyl diethanolamine and diethyl ethanolamine; piperidine; 2-amino - 2 - methyl-1-propanol; 2-amino-1-butanol; methyl piperidine; benzylamine, naphthylamine, aniline, methyl aniline; and compatible mixtures of any two or more thereof.

Only minor amounts of the reaction product of the amine and the phosphate ester are necessary in order to produce a lubricant having the aforementioned superior characteristics. While the preferred concentration is of the order of about 0.1 to 0.2 weight percent in water, concentrations as low as 0.01% and as high as several percent, for instance, 5 to 10%, can be used but such higher concentrations are unnecessary.

Supplemental ingredients for obtaining special effects can be added in minor proportions, if desired, examples of which are, for instance, corrosion inhibitors for certain metals, load support agents, etc.

The invention is further illustrated but not limited by the following examples wherein all percentages reported are by weight.

### Example I

A 0.1% solution in water of the triethanolamine salt of a phosphate ester, prepared by reacting  $P_2O_5$  with a 4 mole ethylene oxide adduct of phenol, was subjected to the Falex Load Test Method to demonstrate load carrying properties. For purposes of comparison, data for an 8 mole ethylene oxide phenol phosphate ester, also as a 0.1% triethanolamine salt solution in water, is included. Briefly, the test employs a Faville LeVally lubricant tester equipped with an automatic loading device, load gauge, torque indicating gauge, brass shear pins, steel journals and steel V bearing blocks. The lubricant is placed in the machine and torque readings are taken at 250 lb. increments until failure occurs or the maximum load of 4500 lbs. is reached. Failure is indicated either by sudden shearing of the brass locking pins or wear occurring at such a rate that the loading ratchet is not able to maintain the load and the load actually decreases. The results are summarized in the following table.

#### FALEX WEAR TEST DATA

Extreme Pressure Load Failure at: 1,750 lbs.; 1,000 lbs.

Conditions:

Temperature: 150° F.

Time: 2 min. each at 250, 500 and 750 lbs., and 15 min. at 1,000 lbs.

| Load (lb.): | Torque (inch-lbs.)                      |                                         |  |
|-------------|-----------------------------------------|-----------------------------------------|--|
|             | Phenol plus 4 mole E.O. phosphate ester | Phenol plus 8 mole E.O. phosphate ester |  |
| 250-----    | 5-5                                     | 13-15                                   |  |
| 500-----    | 7-9                                     | 20-19                                   |  |
| 750-----    | 12-11                                   | 21-5-22                                 |  |
| 1,000-----  | 13-14                                   | 24-23                                   |  |

### EXAMPLE II

#### A

The low foaming characteristics of an illustrative composition of the present invention is demonstrated by the following Ross-Miles Foam Test data wherein the phosphate ester was tested in its free acid form. Comparative data for an 8 mole E.O. phenol adduct phosphate ester and a phosphate ester of an ethoxylated long chain alcohol, also in their free acid form, are included for comparative purposes. All test solutions were 0.1% by weight in water.

#### ROSS-MILES FOAM TEST

| Phosphate ester                        | Mm. of foam |        |        |
|----------------------------------------|-------------|--------|--------|
|                                        | 0 min.      | 1 min. | 5 min. |
| (1) Phenol plus 4 moles E.O.-----      | 5           | 0      | 0      |
| (2) Phenol plus 8 moles E.O.-----      | 25          | 5      | 2      |
| (3) "Antara LS-500" <sup>1</sup> ----- | 70          | 55     | 50     |

<sup>1</sup> A phosphate ester prepared from an ethoxylated long chain aliphatic alcohol and sold under this designation by General Aniline and Film Corp.

#### B

Again, to demonstrate the low foam characteristics of the phosphate esters used in accordance with the present invention, the following Dynamic Foam Test data are

given. This test generally involves stirring 100 ml. of test solution at high speed and measuring the foam volume at equal time intervals. For details of the procedure see Journal of the American Oil Chemists' Society, 31, 254-257 (1954)

#### DYNAMIC FOAM TEST

| 10                               | Phosphate ester | Foam generation rate | Maximum foam volume (5 min. stirring time) |
|----------------------------------|-----------------|----------------------|--------------------------------------------|
|                                  |                 |                      | 15                                         |
| (1) Phenol plus 4 mole E.O.----- |                 | 7.5                  | 15                                         |
| (2) Phenol plus 8 mole E.O.----- |                 | 17.5                 | 45                                         |
| (3) "Antara LS-500"-----         |                 | 20                   | 40                                         |

#### Example III

The triethanolamine salt of the phosphate ester of a 4 mole ethylene oxide adduct of phenol was tested for corrosion inhibition properties. In the test, 4 g. of cast iron chips are placed in 50 ml. of test solution (water solution) for 15 minutes with periodic swirling. At the end of the 15 minute interval, the solution is decanted off and the excess liquid is removed by placing the chips on absorbent paper. The moist chips are then examined visually for rusting.

| 20   | Conc. test solution: | Rusting |
|------|----------------------|---------|
| 0.1% | -----                | Slight. |
| 0.5% | -----                | None.   |
| 1%   | -----                | None.   |
| 2%   | -----                | None.   |

What is claimed is:

1. A lubricant comprising water containing at least about 0.01% by weight of an amine salt of an ester selected from the group consisting of the mono- and di-ester and mixtures thereof of phosphoric acid and an adduct of 1 mole of phenol with from about 1 to about 6 moles of ethylene oxide.

2. A composition according to claim 1, wherein the phosphate ester is selected from the group of esters of the following formulae:



and



where  $n$  is an integer from about 3 to 5.

3. A composition according to claim 1, wherein the amine is a lower molecular weight alkanolamine.

4. A composition according to claim 3, wherein the alkanolamine is triethanolamine.

5. A lubricant composition according to claim 1, containing about 0.1 to about 0.2% of the triethanolamine salt of a phosphate ester selected from the group of esters of the following formulae:



and



where  $n$  is an integer of about 4.

6. A method of effecting lubrication in metalworking operations which comprises applying to the metal surface undergoing working a lubricant in accordance with claim 1.

7. A method of effecting lubrication in metalworking operations which comprises applying to the metal surface undergoing working a lubricant in accordance with claim 5.

## References Cited

## UNITED STATES PATENTS

3,310,489 3/1967 Davis ----- 252—32.5

5 DANIEL E. WYMAN, Primary Examiner

I. VAUGHN, Assistant Examiner

U.S. Cl. X.R.

72—42; 252—49.3